

# UNITED STATES PATENT OFFICE.

BRUCE FORD, OF PHILADELPHIA, PENNSYLVANIA.

## PROCESS FOR MAKING AUTOGENOUS JOINTS.

1,234,699.

Specification of Letters Patent.

Patented July 24, 1917.

No Drawing.

Application filed December 13, 1913. Serial No. 806,405.

*To all whom it may concern:*

Be it known that I, BRUCE FORD, a citizen of the United States, and a resident of Philadelphia, in the county of Philadelphia and State of Pennsylvania, have invented a certain new and useful Process for Making Autogenous Joints, of which the following is a specification.

The principal object of the present invention is to provide an expeditious and satisfactory process for making autogenous joints between lead and copper and the like. Another object of the invention is to provide for casting the lead terminals upon copper wires and bars, such as are used in storage battery connections.

The process consists in first amalgamating the copper with mercury, then placing the amalgamated metal in a mold and casting the lead upon it. The mercury is either volatilized or absorbed by the lead, so that its effect is negligible except that it makes an integral union between the lead and copper, which would not be the case if the copper were not previously amalgamated. In other words, when lead is cast upon copper the union is not satisfactory, but by amalgamating the copper and then casting the lead upon it the union is satisfactory and the mercury does not seem to produce any effect other than bringing about the closeness or perfectness of this union.

A convenient method of amalgamating the copper is to first moisten it with an aqueous solution of caustic, such as caustic soda and to then dip it into the mercury. A vessel containing mercury to the required depth with a solution of caustic on top of the mercury into which the copper is dipped, answers the same purpose. When the copper has been properly amalgamated, for example, in either of the ways mentioned, it is wiped

dry and placed in an appropriate mold. This amalgamated metal is cold when placed in the mold which is advantageous because if it were attempted to place it in the mold hot, the amalgam, or perhaps more accurately, the mercury, would be vaporized or oxidized, and one of the essentials is to avoid oxidation. Thereafter the lead is poured into the mold upon the amalgamated copper and upon cooling it is found that the union between the two is extremely perfect and the mercury appears to have disappeared either by volatilization or possibly absorption by the lead.

What I claim is:

1. The process of making autogenous joints which consists in amalgamating a metal, arranging the cold amalgamated metal in a mold, and casting other molten metal into the mold and upon the amalgam.

2. The process of making autogenous joints between lead and copper which consists in first amalgamating the copper, placing the amalgamating metal while cold in a mold, and casting the lead upon it.

3. The process of making autogenous joints between lead and copper which consists in subjecting the copper to the action of a caustic solution and then dipping it in mercury, wiping the amalgam dry, putting the dry amalgamated copper in a mold, and casting molten lead upon the amalgam in the mold, substantially as described.

4. The process of making autogenous joints between lead and copper which consists in first amalgamating the copper and then casting the lead onto the amalgamated copper.

BRUCE FORD.

Witnesses:

GEO. M. HOWARD,  
L. H. FLANDERS.

Copies of this patent may be obtained for five cents each, by addressing the "Commissioner of Patents, Washington, D. C."